

Aug. 29, 1972

MAKOTO YOSHIDA ET AL  
COLOR PHOTOGRAPHIC LIGHT-SENSITIVE MATERIALS CONTAINING A  
CYAN DYE FOR SILVER DYE BLEACHING METHOD

Filed Sept. 22, 1970

3,687,673



INVENTORS  
MAKOTO YOSHIDA  
SHINICHI IMAI

BY Sughrue, Rothwell, Maw,   
Trim & Macpeak

ATTORNEYS

1

3,687,673

COLOR PHOTOGRAPHIC LIGHT-SENSITIVE MATERIALS CONTAINING A CYAN DYE FOR SILVER DYE BLEACHING METHOD

Makoto Yoshida and Shinichi Imai, Kanagawa, Japan, assignors to Fuji Photo Film Co., Ltd., Kanagawa, Japan

Filed Sept. 22, 1970, Ser. No. 74,342

Claims priority, application Japan, Sept. 22, 1969,

44/75,466

Int. Cl. G03c 1/10

U.S. Cl. 96—99

7 Claims

ABSTRACT OF THE DISCLOSURE

A color photographic light-sensitive material for the silver dye bleaching method comprising a support having thereon a photographic emulsion layer containing a member selected from the group consisting of a cyan dye having the following general formula



wherein X is selected from the group consisting of a halogen atom, a hydroxyl group, an amino group and an anilino group, and wherein Y is a residual group of a compound capable of reacting with the most readily reactive chlorine atom of cyanuric chloride, and the sodium and ammonium salts thereof, is disclosed.

5 dye does not diffuse into other photographic layers and does not adversely affect the photographic properties of the photographic emulsion, such as the formation of fog and desensitization. Still further, it is necessary for the dye formed from such an azo dye to have such properties as desirable absorption spectral characteristics as a cyan dye and a stability to the severe chemical treatments of the silver dye bleaching method, such as development, dye 10 bleaching, and silver bleaching, as well as have sufficient fastness to light, heat, and humidity.

15 Therefore, an object of this invention is to improve the color reproducibility of color photographs by using a cyan dye satisfying the above-described characteristics required for the dye to be used in color photographic light-sensitive materials for the silver dye bleaching method and also having a maximum absorption wave length at the longer wave length side.

20 Another object of this invention is to provide a color

photographic light-sensitive material for the silver dye bleaching method containing an improved cyan dye.

SUMMARY OF THE INVENTION

The objects of this invention can be achieved by incorporating in a color photographic light-sensitive material for the silver dye bleaching method a cyan dye represented 40 by the following general Formula I:



BACKGROUND OF THE INVENTION

(1) Field of the invention

The present invention relates to a color photographic light-sensitive material for the silver dye bleaching method, wherein a cyan dye is incorporated in a photo-sensitive silver halide emulsion layer.

(2) Description of the prior art

Azo dyes are usually used as the cyan dyes in color photographic light-sensitive materials for the silver dye bleaching method. It is necessary that the azo dye be bleached in response to the silver image formed on development to form a positive image of a cyan dye. Therefore, in order that the dye be used for the purpose, the azo group of the dye must be readily reduced and decomposed in response to the amount of silver present, thereby the dye is completely bleached. Also, when the dye is incorporated in a silver halide emulsion, it is necessary that the

55 wherein X represents a halogen atom, a hydroxyl group, an amino group, or an anilino group and Y represents a residual group of a compound capable of being reacted with the first chlorine atom of cyanuric chloride.

DESCRIPTION OF THE INVENTION

60 It is known that the three chlorine atoms of cyanuric chloride can result in a three-step replacement reaction in accordance with the reaction temperatures, that is to say, the first chlorine atom reacts at about 0° C., the second chlorine atom at about 40° C., and the third chlorine atom at about 90° C.

65 Examples of the residual group of a compound which can be reacted with the first chlorine atom of cyanuric chloride, the most readily replaceable chlorine atoms described above are a hydroxyl group, an alkoxy group, an aryloxy group, a mono-substituted amino group, a di-substituted amino group, a nitrogen-containing cyclic group, a sulfoamino group, a thioalkyl group, and the like.

In order to obtain a cyan dye having absorption at a longer wave length region, one of the amino groups of the H-acid which is the nuclei of a cyan dye can be in an unsubstituted state. That is to say, the maximum absorption wave length of an aqueous solution of dye A having the following formula

Dye A:



is 674  $\mu\mu$ , which is almost the same as that of the dye used in this invention. However, because the dye is not substituted at the amino group, the dye diffuses into other photographic layers when it is incorporated in a photographic emulsion layer of a color photographic light-sensitive material. This makes the utilization of the dye in color photographic light-sensitive materials difficult.

Therefore, substitutions of the amino group of the H-acid might provide a diffusion resisting property to the dye. Dye B having the following formula prepared by substituting the amino group of H-acid with, for instance, benzoyl chloride

Dye B



does not diffuse into other photographic emulsion layers when it is incorporated in a photographic emulsion layer of a color photographic light-sensitive material. However, this dye shows no absorption at a longer wave region. Thus, such a type of a diffusion resisting dye is therefore inadequate for a color photographic light-sensitive material. That is to say, the maximum absorption wave length of an aqueous solution of Dye B is 606  $\mu\mu$ , which is extremely shorter than that of the dye used in this invention.

The inventors have investigated a cyan dye in which the amino group of the H-acid is substituted and which has the maximum absorption wave length at the wave length region of as long as possible, and have discovered that the purposes are fulfilled by the dye having the structure shown by general Formula I. In other words, by substituting the amino group of H-acid with an S-triazine group, a cyan dye satisfying the above purposes can be obtained.

The cyan dyes to be used in this invention, for instance dye 1 and dye 2, shown hereinafter, having extremely desirable absorption characteristics as shown in the accompanying drawing, are readily bleached, and have no adverse influence on the photographic properties of a silver halide photographic emulsion when the dye is added to the emulsion. Also, the cyan dyes have sufficient fastness. Thus, the cyan dyes of this invention are quite desirable as cyan dyes for color photographic light-sensitive materials in silver dye bleaching method.

#### DESCRIPTION OF THE ACCOMPANYING DRAWING

The accompanying drawing is a graph showing comparatively the spectral absorption curves of an aqueous solution of two dyes used in the instant invention [Dyes 1 and 2] and an aqueous solution of known dyes [Dyes A and B].

#### DETAILED DESCRIPTION OF THE INVENTION

The cyan dyes of this invention can be used not only for natural color photographic light-sensitive materials

in the silver dye bleaching method but also for color photographic light-sensitive materials used in the silver dye bleaching method for forming single color images and two color images.

The cyan dyes of this invention can be synthesized in the following manner. First, the first chlorine atom of the

three chlorine atoms of cyanuric chloride is replaced with the residual group Y to prepare a 2-Y substituted-4,6-dichloro-S-triazine. Then, the N-substituted H-acid is synthesized by utilizing the reaction of the second chlorine atom of the substituted triazine prepared above and the amino group of H-acid. Then the N-substituted H-acid is reacted with the diazo component of a monoazo dye to obtain the cyan dye.

As the cyan dyes to be used in this invention, suitable ones are those having, for example, the following structures although they are not limited to them only. In addition, the sulfone group of each of the cyan dyes shown

below can be substituted by a sodium atom, potassium or an ammonium group. In the structural formulae shown below, the following grouping is denoted as A:



45

(1)



50

(2)



60

(3)



## 5

(4)



(5)



(6)



Now, typical examples of the synthesis of the cyan dyes of this invention are illustrated below.

## SYNTHESIS 1

## Synthesis of the dye having structural Formula 2

(1-1) Synthesis of diazo component.—198 parts by weight of 1-amino-2,5-dimethoxy-4-nitrobenzene are diazotized in a strong hydrochloric acid suspension. The diazotized liquid is added to 423 parts by weight of a solution of 1-benzoylaminoo-8-hydroxynaphthalene-3,6-disulfonic acid made alkaline with sodium carbonate to cause coupling. By reducing the nitroazo dye thus obtained with sodium sulfide in an alkaline solution, the corresponding amino-azo dye is obtained and then the dye is isolated (see the specification of Japanese patent publication No. 25,768/1964).

(1-2) Synthesis of coupling component.—A solution of 18.5 parts of cyanuric chloride in 100 parts of acetone is added in a mixture of 300 parts of water and 300 parts of ice and then 6.7 parts of aqueous ammonia having a specific gravity of 0.89 are added to the mixture at temperatures of lower than 0° C. When the ammonia is consumed, 6.7 parts of aqueous ammonia are further added to the system, and the mixture is stirred for about 1 hour at temperatures below 0° C. Thereafter, the solution is acidified slightly by adding 1-N hydrochloric acid.

A solution of 36.3 parts of sodium 1-amino-8-naphthol-3,6-disulfonate in 200 parts of water is added to the suspension of 2-amino-4,6-dichloro-S-triazine prepared above. The solution is heated for 45 minutes at 55° C. and then the solution is further stirred at the same temperature until the 1-amino-8-naphthol-3,6-disulfonic acid is consumed. Thereafter, the solution is neutralized by adding an aqueous 2 N sodium carbonate solution and then cooled, thereby the desired material is deposited. The product is then collected by filtration and dried.

(1-3) Synthesis of dye (2).—The diazonium solution of the diazo component obtained in synthesis (1-1) is coupled with the coupling component obtained in synthesis (1-2) in an aqueous pyridine solution at 20° C. The dye obtained above is dissolved again in water and purified by a repeated salting out operation until the purple impurities are completely removed. Then, the product solution is subjected to a salting out by sodium acetate. The precipitates are collected by filtration, washed with ethanol and dried.

6  
SYNTHESIS 2

## Synthesis of the dye of structural Formula 1

The same procedure as used in Synthesis (1-2) described above is followed using 2-hydroxy-4,6-dichloro-S-triazine to obtain a coupling component, which is coupled with the diazo component obtained in synthesis (1-1) described above. Thereafter, by following the same procedure as used in Synthesis (1-3) described above, the dye having the structural Formula I is obtained.

## SYNTHESIS 3

## Synthesis of the dye of structural Formula 3

2-hydroxy-4,6-dichloro-S-triazine is reacted with 1-amino-8-naphthol-3,6-disulfonic acid as in Synthesis (1-2) described above and then a coupling component is obtained using the method of hydrolyzing the residual chlorine of chloro-S-triazine by heating in a weak hydrochloric acid solution. Thereafter, the coupling component is coupled with the diazo component obtained in Synthesis (1-1) and by treating the product by the same procedure as used in Synthesis (1-3), the dye having the Formula 3 is obtained.

The invention is now explained in greater detail by reference to the following examples.

## EXAMPLE 1

1 g. of the cyan dye shown by the structural Formula 2 was dissolved in 100 ml. of a 5% aqueous sodium hydroxide solution and a mixture of 80 ml. of the dye solution thus obtained and 100 g. of a silver bromide emulsion (containing about 30 g. of silver bromide per kilogram of the emulsion) was coated on a film base. The light-sensitive film prepared was exposed under a step wedge and then developed for 10 minutes using a developing solution having the following composition:

|                                                     | G. |
|-----------------------------------------------------|----|
| 40 N-methyl-p-aminophenol 1/2 sulfate               | 2  |
| 40 Anhydrous sodium sulfite                         | 30 |
| 40 Hydroquinone                                     | 8  |
| 40 Sodium carbonate                                 | 20 |
| 40 Potassium bromide                                | 4  |
| 40 Water added to make the total volume to 1 liter. |    |

The film developed was then washed with water and fixed for 4 minutes using a solution having the following composition:

|                                 | G.  |
|---------------------------------|-----|
| 50 Anhydrous sodium thiosulfate | 350 |
| 50 Anhydrous sodium sulfite     | 10  |

50 Water added to make the total volume to 1 liter.

The film was then washed with water, hardened, using a 4% aqueous formaldehyde solution, washed with water, and then processed for 15 minutes using a dye bleaching bath having the following composition:

|                                                     |      |      |
|-----------------------------------------------------|------|------|
| 60 Thiourea                                         | g--  | 60   |
| 60 Potassium bromide                                | g--  | 30   |
| 60 Concentrated hydrochloric acid                   | ml-- | 30   |
| 60 2-amino-3-hydroxyphenazine                       | g--  | 0.01 |
| 60 Water added to make the total volume to 1 liter. |      |      |

The film was washed with water and then treated using a silver bleaching bath having the following composition:

|                                   |      |     |
|-----------------------------------|------|-----|
| 65 Crystalline copper sulfate     | g--  | 100 |
| 65 Concentrated hydrochloric acid | ml-- | 100 |

65 Water added to make the total volume to 1 liter.

The film was washed with water, fixed again using the fixing bath having the composition shown above, washed further with water, and dried.

70 Using the above-described treatments, a completely bleached cyan image was formed at the highlight portion. The image produced was suitable as the cyan component image of a multi-color type light-sensitive material for the silver dye bleaching method.

## EXAMPLE 2

The same procedure as used in Example 1 was followed using the cyan dye shown by the structural Formula 1 and a cyan image was obtained. The highlight portion of the image was completely bleached and the image was suitable as the cyan component image of a multi-color type light-sensitive material using a silver dye bleaching method.

## EXAMPLE 3

The same procedure as used in Example 1 was followed using the cyan dye having the structural Formula 3 and a cyan image was obtained. The highlight portion of the color image was completely bleached and was suitable as

wherein X is selected from the group consisting of a halogen atom, a hydroxyl group, an amino group and an anilino group and wherein Y is a residual group of a compound capable of reacting with the most readily reactive chlorine atom of cyanuric chloride selected from the group consisting of a hydroxyl group, an alkoxy group, an aryloxy group, an amino group, a mono-substituted amino group wherein the substituent is an aryl group, a nitrogen-containing saturated cyclic ring group having 6 members, 5 a sulfoamino group, a thioalkyl group, and the sodium and ammonium salts thereof.

10 2. The color photographic light-sensitive material according to claim 1, wherein said cyan dye has the following formula



the cyan component image of a multi-color type light-sensitive material using a silver dye bleaching method.

3. The color photographic light-sensitive material according to claim 1, wherein said cyan dye has the following formula



What is claimed is:

1. A color photographic silver halide light-sensitive material for the silver dye bleaching method comprising

4. The color photographic light-sensitive material according to claim 1, wherein said cyan dye has the following formula



a support having thereon a photographic emulsion layer containing a member selected from the group consisting of a cyan dye having the following general formula:



5. The color photographic light-sensitive material according to claim 1, wherein said cyan dye has the following formula



6. The color photographic light-sensitive material according to claim 1, wherein said cyan dye has the following formula



7. The color photographic light-sensitive material according to claim 1, wherein said cyan dye has the following formula



## References Cited

UNITED STATES PATENTS

- 3,178,291 4/1965 Mory et al. ----- 96-99  
3,211,554 10/1965 Dreyfuss ----- 96-99

J. TRAVIS BROWN, Primary Examiner

U.S. Cl. X.R.

96—73; 260—153